

(No Model.)

W. WILMINGTON.

METHOD OF CASTING CAR WHEELS.

No. 363,444.

Patented May 24, 1887.



*Witnesses:*

*A. Ruppert.*

*C. B. Thompson.*

*Inventor:*

*William Wilmington,  
by G. W. J. Howard,  
Attest.*

# UNITED STATES PATENT OFFICE.

WILLIAM WILMINGTON, OF TOLEDO, OHIO.

## METHOD OF CASTING CAR-WHEELS.

SPECIFICATION forming part of Letters Patent No. 363,444, dated May 24, 1887.

Application filed March 15, 1887. Serial No. 231,002. (No model.)

*To all whom it may concern:*

Be it known that I, WILLIAM WILMINGTON, of Toledo, in the county of Lucas and State of Ohio, have invented certain new and useful 5 Improvements in the Art of Casting Car-Wheels, of which the following is a specification, reference being had to the accompanying drawing, and to the letters of reference marked thereon.

- 10 This invention is an improvement in the art of casting chilled-tread cast-iron car-wheels; and it consists in a novel process or method of combining with molten chill-hardening cast-iron during certain stages in the casting of the 15 wheel the commercial metalloids of ferro-manganese (or its equivalent rich spiegeleisen) and rich ferro-silicon, (or its equivalent silicon-spiegel,) the same being introduced during the continuous inflow of molten iron into the mold.
- 20 The object of the invention is to restore or give to the molten iron during the different stages of casting the quantities required for the different parts of the wheel of carbon, silicon, and manganese, these elements having 25 been more or less removed by previous melt- ings of the iron.

Heretofore different patents of the United States have been granted to me upon methods of casting iron car-wheels, the inventions of 30 which consist in incorporating, in varying quantities, rich and finely-powered ferro-manganese of commerce with molten cast-iron composing the wheel by placing the same in the stream of iron flowing from the pouring-ladle 35 or directly into the basin of the mold during the casting of the wheel; and an application (Serial No. 222,600) for a patent for an improvement in casting wheels has recently been allowed to me, which improvement consists in 40 incorporating, in varying quantities, during the casting of the wheel, rich and finely-pow- dered ferro-silicon of commerce with molten chill-hardening cast-iron. These methods pro- 45 duce beneficial effects upon the iron compos- ing certain parts of the car-wheel, but not to the requisite extent when the production of a cheap wheel from low-priced and partially-decarbonized high chill-hardening cast-iron is desired, from causes which may be stated as 50 follows:

When, in accordance with my said patented methods, molten cast-iron very high in chill-

hardening qualities first enters the mold of a wheel on filling the depression in the drag wherein is formed a part of the hub of the 55 wheel, it loses its heat rapidly by coming in contact with the sides of the lower end of the cold central core and moist sand of the mold. It will be remembered that the ferro-manganese is added in comparatively greater quantities at the later stages of the pouring, and consequently, there not being a sufficient quantity of said substance in combination with the first inflow of iron to modify it to the proper degree on its contact with the central core, the 65 chill-hardening properties of the iron leave the metal, when cold, around the axle-opening dense and hard, making it at times a difficult matter to bore the wheel correctly.

In the practice of my present invention I 70 prefer to melt in a cupola in the common man- ner old or condemned cast-iron car-wheels or other low-priced partially-decarbonized chill-hardening cast-irons, which, by repeated melt- 75 ings, have been more or less deprived of their carbon, silicon, and manganese, leaving the iron high in chill-hardening properties, which qualities produce the best results in carrying out my present method of casting wheels.

The object of my present improvement is 80 therefore to obviate the difficulty arising from the employment of low-priced and partially-decarbonized cast-irons, the use of which is necessary to produce a cheap wheel. This iron being deficient in the proper proportions 85 of carbon, silicon, and manganese, that must compose certain portions of the wheel to pre- vent undue hardness of the iron at the hub of the wheel, I incorporate the proper quantities of the elements contained in rich ferro-manganese and rich ferro-silicon (or their described equivalents) with the molten iron forming dif- 90 ferent parts of the wheel during the continu- 95 ous pouring or casting of the same.

In the drawing is shown a cross-section of 95 a mold for a single-plated car-wheel.

A represents the basin of the mold.

B B show two or more openings in the bot- 100 tom of the basin leading directly into the mold.

C shows a vertical opening through the bot- 105 tom of the basin and the central core of the mold.

D D represent four or more horizontal out- 110 lets leading outward from the vertical open-

ings in the central core into the hub part of the mold.

The molten iron being drawn into a reservoir-ladle, from this iron trial-pieces are cast.

5 The brittleness of these pieces on fracture determines the quantities of ferro-manganese and ferro-silicon (or their equivalents) that will be required to produce the desired effects upon the iron composing the different parts of the wheel. The wheel is afterward cast in the ordinary manner by the continuous pouring of the molten iron, except that a distinctive method or process of operation is also employed, as follows: At the time or immediately after the molten iron enters the mold I place in the stream of molten metal flowing from the pouring-ladle, with a suitable sheet-metal scoop, rich and finely-powdered ferro-manganese and rich and finely-powdered ferro-silicon, using the same scoop for the two substances, which are at first not mixed or combined, the ferro-manganese being discharged first from the scoop gradually into the stream of molten iron or directly into the basin of the 15 mold during about two-thirds of the filling of the mold. At this stage in the casting of the wheel a mixture of ferro-manganese and ferro-silicon is discharged from the scoop into the stream of molten iron passing from the ladle 25 or directly into the basin of the mold, the same continuing until the mold is filled.

The effects produced by this method of casting car-wheels are as follows: The powdered ferro-manganese, coming in contact with the molten iron in the stream or in the basin, is quickly melted by the inherent heat of the iron, and combining with the iron adds strength to the same. The first of this iron thus mixed with ferro-manganese, entering the mold 35 through the openings in the bottom of the basin, fills that part of the mold in which is formed the hub of the wheel, and then fills those parts of the mold in which are formed the arms, the plate, and the parts of the tread 40 of the wheel most subject to wear. The iron, at this stage of casting the wheel, has but a small quantity of ferro-manganese mixed with it, which secures durability to a part of the tread of the wheel, the same being made dense 45 and hard. A part of the continued inflow of the iron, having mixed with it the ferro-manganese, being discharged from the horizontal openings in the central core into the hub part of the mold, and imparting heat to the core 50 and the sand of this part of the mold, the now inflowing iron, having in combination ferro-manganese and ferro-silicon, will displace from the central core the iron first poured, and com-

ing in contact with the heated central core and the sand, the cooling of the molten iron 55 will be prolonged, which will aid the ferro-silicon in preventing this iron from becoming dense and hard.

To produce a cheap, strong, and durable chilled-tread wheel from the qualities of iron 60 described, I use about one pound of finely-powdered eighty per cent. ferro-manganese and about three pounds of finely powdered nine per cent. ferro-silicon.

In the use of some varieties of irons I find 65 it advantageous to increase the quantity of free carbon in the ferro-silicon by adding, in combination with the same, free or graphitic carbon of commerce in the desired quantities. The metalloids of ferro-manganese and ferro-silicon and their equivalents being articles of 70 artificial production, their quality is not always correctly given in commerce. Therefore I do not confine myself to the use of the exact 75 quantities of the same specified, but use such quantities as are found to produce the best effects upon the iron composing the different parts of the wheel; nor do I confine myself to any particular stage in the casting of the wheel before commencing the incorporation with the 80 iron of the combined metalloids of ferro-silicon and ferro-manganese or their equivalents; but I commence the incorporation of these metalloids therewith at a stage in the filling 85 of the mold shown by practice to produce the best results in the wheel being cast. I am thus enabled to produce a cheap and efficient cast-iron car-wheel having a hard and durable tread, while the hub and inner plate parts are 90 soft and strong.

95 What I claim is—

The method of casting chilled-tread cast-iron car-wheels, which consists in first filling a portion of the mold with molten chill-hardening cast-iron, the same having combined 100 with and disseminated through it in a melted state a quantity of ferro-manganese of commerce, then filling the remainder of the mold by the continuous inflow of the same quality of molten cast-iron having combined with and 105 disseminated through it in a melted state a mixture of ferro-manganese and ferro-silicon of commerce in varying quantities, substantially as described, and for the purpose set forth.

110 In testimony whereof I have hereunto set my hand and seal this 17th day of February, 1887.

WILLIAM WILMINGTON. [L. S.]

Witnesses:

ALEXANDER WEBER,  
LINCOLN HAYS.